

## 1

3,227,556  
PHOTOSENSITIVE ELEMENTS CONTAINING  
FORMAZANS

Gene L. Oliver and John W. Gates, Jr., Rochester, N.Y.,  
assignors to Eastman Kodak Company, Rochester,  
N.Y., a corporation of New Jersey  
No Drawing. Filed Dec. 11, 1962, Ser. No. 243,756  
8 Claims. (Cl. 96—109)

This invention relates to use of formazans in photosensitive elements for photography.

Formazans that are useful according to the present invention are a class of compounds having the formulas



and



wherein each of  $\text{R}_1$  and  $\text{R}_2$  represents a member selected from the group consisting of aryl and substituted aryl.  $\text{R}_3$  represents a member selected from the group consisting of aryl, substituted aryl, nitro, alkyl containing 1 to 18 carbon atoms, and H and X represents dialkoxydiphenyl.

An object of the present invention is to provide photographic elements for use in photography comprising at least one layer which contains a formazan compound of the class defined above.

Spectra of compounds of the class defined above are characterized by rather broad absorption bands in the visible region. Changes of substituent groups  $\text{R}_1$ ,  $\text{R}_2$  and  $\text{R}_3$  in the class of compounds cause variation of absorption maxima over a considerable range. This is illustrated in Table 1 which shows absorption maxima of some typical formazans.

Table 1

|                                                                     | Max.,<br>$\text{m}\mu$ | Reference                                             |
|---------------------------------------------------------------------|------------------------|-------------------------------------------------------|
| A. 1,5-diphenyl-3-ethoxycarbonyl formazan.                          | 440                    | J. pr. Chem. 65, 123 (1902).                          |
| B. 1,5-diphenyl-3-nitroformazan.                                    | 444                    | J.A.C.S. 65, 2390 (1943).                             |
| C. 3,5-diphenyl-1-phenylazophenyl formazan.                         | 510                    | J. Chem. Soc. 3881 (1953); J. Chem. Soc. 1565 (1954). |
| D. 1,1'-(3,3'-dimethoxy-4,4'-biphenylene)bis(3,5-diphenylformazan). | 598                    | Annalen 581, 16 (1953).                               |
| E. 1,3,5-triphenyl formazan.                                        | 483                    | Chem. Revs. 55, 446 (1955).                           |
| F. 1-(4-acetamidophenyl)-3,5-diphenyl formazan.                     |                        |                                                       |

According to the present invention, formazans of the class defined above are incorporated in at least one layer of a photosensitive element for use in photography.

A preferred embodiment of the invention is a photographic element comprising a photosensitive silver halide emulsion layer which has incorporated therein an antifogging agent consisting of at least one formazan compound of the class defined. Following are examples which describe in more detail this preferred embodiment.

## EXAMPLE 1

A high-speed, sulfur and gold sensitized bromoiodide emulsion was prepared and coated upon a cellulose acetate film support by conventional procedures. For a control sample, no formazan was added to the emulsion. For a test sample, triphenylformazan was added to the

## 2

emulsion prior to coating in a proportion of 30 mg. per mole of silver in the emulsion. Silver coverage was 432 mg. per sq. ft. and gelatin coverage was 978 mg. per square foot. The control and test samples were then exposed on an Eastman 1B sensitometer by conventional procedure and then processed for five minutes in Kodak DK-50 photographic developer. The samples were then fixed, washed and dried. The control sample had relative speed of 100 and fog density of 0.18. The test sample had relative speed of 71 and fog density of 0.17.

Control and test samples were prepared as just described but were incubated for one week at 120° F., 50% relative humidity before exposure and development. The control had relative speed of 59, fog density of 0.42. The test sample had relative density of 65, fog density of 0.27.

## EXAMPLE 2

Control and test samples were prepared and tested as in Example 1 but with various formazans added before coating as shown in Table 2. For these samples silver coverage was 460 mg. per sq. ft. and gelatin coverage was 1.04 gm. per sq. ft. The letter reference to the formazan antifogging corresponds to letter enumeration in Table 1.

Table 2

| 30 | Sample No.    | Formazan<br>Antifog-<br>gant<br>(Table 1) | Formazan<br>Conc.,<br>Mg. per<br>Mole Ag | Exposed Fresh          |                | Exposed After<br>Incubation |                |
|----|---------------|-------------------------------------------|------------------------------------------|------------------------|----------------|-----------------------------|----------------|
|    |               |                                           |                                          | Rela-<br>tive<br>Speed | Fog<br>Density | Rela-<br>tive<br>Speed      | Fog<br>Density |
| 35 | Control (1-6) |                                           | 0                                        | 100                    | .16            | 29.5                        | .49            |
| 1  | A             | 30                                        | 52                                       | .10                    | .23            | .36                         |                |
| 2  | B             | 30                                        | 42                                       | .08                    | .16            | .38                         |                |
| 3  | C             | 3                                         | 43                                       | .09                    | .17            | .39                         |                |
| 4  | D             | 9                                         | 43                                       | .09                    | .19            | .35                         |                |
| 5  | E             | 3                                         | 67                                       | .10                    | .28            | .36                         |                |
| 6  | F             | 30                                        | 43                                       | .10                    | .23            | .37                         |                |
| 30 | Control (7-9) |                                           | 0                                        | 100                    | .28            | -----                       | .65            |
| 7  | F             | 3                                         | 71                                       | .25                    | -----          | .45                         |                |
| 8  | F             | 30                                        | 71                                       | .25                    | -----          | .42                         |                |
| 9  | F             | 3,000                                     | 50                                       | .24                    | -----          | .39                         |                |

Formazans of the class defined are effective antifogging agents when incorporated at concentrations from about 3 to about 3000 milligrams per mole of silver in silver halide layers.

Although the examples show photographic elements having only one photosensitive silver halide emulsion layer, this invention includes elements having more than one photosensitive emulsion layer, for example color films, in which at least one of such layers contains a formazan of the class defined. In some embodiments of the invention it may be desirable to employ a mixture of the formazans defined above as an antifogging agent for silver halide films.

These formazans have other utility in photographic films and plates in addition to their use as antifogging agents in the photosensitive emulsion layer, for example formazans are useful dyes for filter and antihalation layers.

60 The invention has been described with reference to certain preferred embodiments, but it will be understood that variations and modifications can be made within the scope of the invention defined in the following claims.

We claim:

65 1. A photosensitive element for use in photography comprising a photosensitive silver halide emulsion layer which contains as an antifogging agent at least one formazan compound having the formula selected from the group consisting of



and



wherein each of R<sub>1</sub> and R<sub>2</sub> represent a member selected from the group consisting of aryl and substituted aryl, R<sub>3</sub> represents a member selected from the group consisting of aryl, substituted aryl, alkoxy, nitro, alkyl containing 1 to 18 carbon atoms, and H and X represents dialkoxy biphenylene.

2. A photosensitive element as defined in claim 1 wherein the concentration of formazan compound in said emulsion layer is in the range from 3 to 3000 milligrams per mole of silver in the layer.

3. A photosensitive element as defined in claim 1 wherein said formazan compound is 1,5-diphenyl-3-ethoxycarbonylformazan.

4. A photosensitive element as defined in claim 1 wherein said formazan compound is 1,5-diphenyl-3-nitro-20 formazan.

5. A photosensitive element as defined in claim 1 wherein said formazan compound is 3,5-diphenyl-1-p-phenylazophenylformazan.

6. A photosensitive element as defined in claim 1 wherein said formazan compound is 1,1'-(3,3'-dimethoxy-4,4'-biphenylene)bis(3,5-diphenylformazan).

7. A photosensitive element as defined in claim 1 wherein said formazan compound is 1,3,5-triphenylformazan.

10 8. A photosensitive element as defined in claim 1 wherein said formazan compound is 1-(4-acetamido-phenyl)-3,5-diphenylformazan.

#### References Cited by the Examiner

#### UNITED STATES PATENTS

|           |        |               |       |        |
|-----------|--------|---------------|-------|--------|
| 2,160,907 | 6/1939 | Richardson    | ----- | 96—84  |
| 3,050,393 | 8/1962 | MacDonald     | ----- | 96—84  |
| 3,071,465 | 1/1963 | Dersch et al. | ----- | 96—109 |

15 NORMAN G. TORCHIN, Primary Examiner.